

1

2,714,074

## METHOD OF MAKING DIFFERENT COLORED MARKS WITH A SINGLE FLUID

Barrett K. Green, Dayton, Ohio, assignor to The National Cash Register Company, Dayton, Ohio, a corporation of Maryland

No Drawing. Continuation of abandoned application Serial No. 60,405, November 16, 1948. This application May 28, 1952, Serial No. 290,556

3 Claims. (Cl. 117—45)

This invention relates to a method of making different colored marks with a single fluid and more particularly pertains to a liquid containing an ink and a color-forming reactant to be used in conjunction with sensitized and unsensitized record material, said fluid, when applied to unsensitized record material, without visually perceptible delay making a permanently stable color mark thereon by reason of the intrinsic color of the ink, and, when applied to sensitized record material, without visually perceptible delay making a permanently stable differently colored mark thereon by reason of the intrinsic color of the ink blending with the color produced in the color-forming reactant on contact with the sensitized record material.

This is a continuation of my application Serial No. 60,405, filed November 16, 1948, now abandoned.

Since it is within the purview of this invention to use color-forming reactants which are either colorless or colored in the initial condition but which change to another color when coming into contact with sensitized record material, the color of the ink may, in the event the color-forming reactant in the fluid has an initial color, be modified by the color of the color-forming reactant in its initial state before a color reaction occurs.

The process includes the application of the fluid to the record material in any manner, such as by brushing, spraying, spotting, or printing. A fluid carrier for applying the fluid is described in my application Serial No. 60,642, filed November 18, 1948, and a porous printing member for applying the fluid is described in my application Serial No. 60,404, filed November 11, 1948. Said applications Serial No. 60,404 and Serial No. 60,642 have been abandoned after the filing of a continuation application, Serial No. 209,981, on February 8, 1951. However, I contemplate the use of my process in letter-press and offset printing, hand-stamping, stencilling, painting, and like operations.

A fluid is first prepared containing a selected ink and a selected color-forming reactant, and then the dual-purpose fluid is applied selectively to unsensitized or sensitized receiving material. The ink may be of either the dye or the pigment type, and the color-forming reactant may be a liquid or a solid which is dissolved so as to form a fluid mixture with the ink. The ink, if it is itself a fluid, may be used as a solvent or vehicle for the color-forming reactant or vice versa. In any instance, it is proposed that the color-forming reactant will remain in its unreacted state in the fluid or as marks of dried fluid unless it comes into contact with the sensitized material.

Because the invention is primarily important in the field of record keeping, where the distinctiveness of the two different colors must be maintained, it is important to have the color reactant in the fluid of such a character that it will not change to the reacted colored form on unsensitized record material because of the presence of light or air, even though exposed thereto for protracted periods of time, because if exposure to air or light, only, changes the color of the fluid-carried color reactant, then,

2

in time, the color of the marks on the unsensitized record material would become the same as the color of the marks on the sensitized record material. The fluid-carried color reactants disclosed in this specification are not changed to the colored form by mere exposure to light or air and, hence, are free from the defects of air-oxidizable leuco vat dyes, which are sometimes used in conjunction with inks in the so-called fraud-preventing inks, such as those described in United States Patent No. 2,068,204, which issued on the application of B. W. Smith.

As the process finds its most important use in printing, a preferred embodiment of the invention as employed in that art is disclosed, using as an example the application of the fluid to record material, sensitized in selected areas, by means of an ordinary rubber hand stamp having type faces of rubber or artificial rubber, which may be coated with the fluid in any manner, as by pressing the stamp against an absorbent pad previously impregnated with the fluid.

Therefore, it is an object of this invention to provide a method of making different colored marks, color-stable in the presence of light or air, with a single fluid.

Another object of the invention is to provide such a method in which the ink color blends with the color formed by the color-forming reactant, on reaction, to produce a color distinctive from that of the ink and unreacted color-forming reactant.

With these and other objects in view, the invention will be described as embodied in a preferred and other forms, showing its utility and novelty.

In describing the preferred embodiment, the method will be assumed to be used in conjunction with paper having sensitized and unsensitized areas. The sensitization is carried out by application to the paper of fine particles of attapulgite, sometimes known as Attapulgus clay, which is white and ideally suited as a paper coating in the manner that other clays are ordinarily used. This attapulgite may be applied to the paper by use of paper coating starch in the following manner: Twenty per cent., by weight, of paper coating starch in water is cooked at 200 degrees Fahrenheit for fifteen minutes and, after cooling, adding to one part, by weight, of the cooked starch four parts, by weight, of a dispersion of one part, by weight, of attapulgite in three parts, by weight, of water. This coating material is applied to paper, on selected areas, at room temperature, and dried. The recommended thickness of the coating, .0005 of an inch, may be varied considerably. The preferred fluid is made by dissolving three per cent., by weight, of crystal violet lactone, which is 3,3 bis(p-dimethylaminophenyl) 6-dimethylamino phthalide, having the structure



and three per cent., by weight, of the red dye Sudan III, which is



in 94 per cent., by weight, of chlorinated diphenyl of 48 per cent., by weight, chlorine content. The fluid is then ready to be absorbed in a stamp pad, transferred to the stamp, and applied by the stamp to sensitized or unsensitized areas of the paper, as desired. This fluid is normally red and will make a red print when applied by the stamp to unsensitized record material but will make a very dark purplish print when applied to record material sensitized by the attapulgite. The red and the dark purplish prints appear without visually perceptible delay when the ink is applied to the record material. Crystal violet lactone may be produced by a method described in United States Patent No. Re. 23,024, which issued on the application of Clyde S. Adams.

There may be substituted for the crystal violet lactone of the preferred embodiment other color-forming reactants which are considered equivalents of that compound, which have a normally colorless state, and which assume a color, without visually perceptible delay, when in adsorption contact with attapulgite.

Among these substitutes may be mentioned:

1. Malachite green lactone, which is 3,3 bis (p-diethylaminophenyl) phthalide, having the structure



producing a green color,

2. The compound 3,3 bis(p-diethylaminophenyl)-6-diethylamino phthalide, having the structure



producing a dark blue color,

3. The compound Michler's Hydrol, which is bis(p-dimethylaminophenyl) methanol, having the structure



producing a dark blue color,

4. The methyl ether of Michler's Hydrol, which is bis(p-dimethylaminophenyl) methoxy-methane, having the structure



producing a dark blue color,

5. The compound 3,3 bis(p-diethylaminophenyl) phthalide, having the structure

5



10

15 producing a blue-green color,

6. The compound 3,3 bis (p-methylaminophenyl) phthalide, having the structure

20



25

30 producing a bright blue color,

7. The compound 3,3 bis(p-ethylaminophenyl) phthalide, having the structure

35



40

45 producing a dark blue color,

8. The compound 3,3 bis(p-n-dipropylaminophenyl) phthalide, having the structure

50



60 producing a blue-green color; and many others.

Following are compounds which are considered equivalents of crystal violet lactone and the compounds mentioned in paragraphs numbered 1 to 8, but which have a color in their normal state but assume another color on contact with attapulgite.

9. The compound 2,4 bis[p-(p-dimethylaminoazo) anilino]-6-hydroxy sym. triazine, having the structure

70



75



which is normally yellow but reacts to produce a bluish-gray color and may be used with red dye ink.

10. The compound o-hydroxybenzalacetophenone, having the structure



which normally is of a light yellow color and produces, on reaction, a reddish-yellow color, such being suitable for use with blue dye to produce a green mark on sensitized paper and a purple mark on unsensitized paper.

The above list is far from being exhaustive but gives a wide choice of color reactants.

In place of attapulgite, color reactants 1 to 8 react with halloysite, magnesium trisilicate, and sodium aluminum silicate zeolite material, all suitable for making recording surfaces and all to be considered equivalents of attapulgite. Color reactants 9 and 10, additionally, react with bentonite and halloysite. The sensitized surface may be prepared by binding such sensitizing material in any way, as by adhesives or paints which do not mask the surface of the particles, so that they remain available to the fluid-carried color-forming reactant applied thereto.

I consider as other equivalents of the color-reactant crystal violet lactone, in addition to those specifically recited, any color-reactant compound that may be carried in a liquid vehicle, which compound is color-stable in light or air in the uncolored or unreacted form in which it is present in the unapplied printing fluid, which is color-stable on unsensitized record material in the presence of light or air, but which will turn to a colored form on contact with record material sensitized as specified, without visually perceptible delay, and remain color-stable in the colored form in the presence of light or air. I do not consider compounds of the vat dye class disclosed in the before-mentioned United States Patent No. 2,068,204, which issued on the application of B. W. Smith, as equivalents of crystal violet lactone, because exposure of those vat dye compounds in the so-called leuco or "unoxidized" state to light and air results in their turning to the same colored oxidized form, whether they are on unsensitized record material or on sensitized record material. Moreover, the compounds mentioned in the aforesaid Smith patent will not form color on any of the oxidizing materials disclosed in said Smith patent without visually perceptible delay even in the presence of strong sunlight, the oxidation to the colored form taking at least several hours.

I consider as equivalents of the color-reactant attapulgite, in addition to those compounds and minerals specifically recited, solid particulate chemical compounds and minerals which, without visually perceptible delay, cause a color change in the color-reactant crystal violet lactone, or its equivalents in the printing fluid, on contact therewith, which are substantially inert as to record material, and which are substantially white or colorless.

The embodiments of the invention disclosed produce marks that usefully are color-stable to the aging influence of light and the atmosphere. The inks are stable in color on both the unsensitized and sensitized areas of the associated record material. The color reactant in the applied fluid is stable to light and atmospheric aging in the unreacted condition on the unsensitized portions of the record material and likewise stable in the reacted color condition on the sensitized portions of the record material.

While the action of the ink and color-forming reactant is best carried out when the ink is of the dye type which will not mask the color produced by the color-forming reactant, the use of pigments in the ink is contemplated if such are selected so as not to mask the color produced by the color-forming reactant material.

It will be apparent that the sensitized and unsensitized materials may be separate entities and not merely areas on a single unitary surface.

It will be obvious that the invention may be carried out by the use of other materials than those mentioned, and, therefore, the invention is claimed broadly.

What is claimed is:

1. The method of making, by use of a single marking fluid, marks of one color on unsensitized record material and marks of another color on record material sensitized with particles of attapulgite, including the step of applying, according to the required configuration to form the marks, to the unsensitized record material and to the sensitized record material, as desired, a colored marking fluid including as a component thereof the normally substantially colorless color reactant 3,3 bis(p-dimethylaminophenyl) 6-dimethylamino phthalide, having the structure



and which is stable to light or air on the unsensitized record material, but turns dark blue, without visually perceptible delay, upon coming into contact with record material sensitized with attapulgite, whereby marks made on unsensitized record material are distinctively different in color from marks made on sensitized record material.

2. The method of printing data in different colors in different areas on record material, with a single fluid, so that data printed in one area is different in color from that printed in another area which has been sensitized by having had applied thereto particles of attapulgite, including the steps of printing data in the sensitized area and in the unsensitized area, as desired, with a colored marking fluid containing, as one ingredient the colorless color-reactant, 3,3 bis(p-dimethylaminophenyl) 6-dimethylamino phthalide, having the structure



and which is normally substantially colorless and stable in light or air on the unsensitized area of the record material but which turns dark blue, without visually perceptible delay, on coming into contact with the area of the record material sensitized with attapulgite, whereby marks made on sensitized areas are distinctively colored differently from marks made on unsensitized areas.

3. The method of making marks of different color on a single piece of record material, by use of a single marking fluid, including the steps of preparing marking-fluid-receiving record material by sensitizing selected areas of the record material by applying thereto particles of attapulgite; preparing a marking fluid having a normal color and having therein a substantially colorless fluid vehicle in which has been dispersed 3,3 bis(p-dimethyl-

aminophenyl) 6-dimethylamino phthalide, having the structure



and selectively applying the fluid to sensitized and unsensitized areas of the record material, as desired.

## References Cited in the file of this patent

## UNITED STATES PATENTS

|    |           |          |       |               |
|----|-----------|----------|-------|---------------|
| 5  | 2,068,204 | Smith    | ----- | Jan. 19, 1927 |
|    | 2,337,737 | Champion | ----- | Dec. 28, 1943 |
|    | 2,348,128 | Groak    | ----- | May 2, 1944   |
| 10 | 2,474,084 | Adams    | ----- | June 21, 1949 |
|    | 2,548,366 | Green    | ----- | Apr. 10, 1951 |